

[54] SLOW FADE INOCCULANT AND A  
PROCESS FOR THE INOCCULATION OF  
MELTED CAST IRON

[75] Inventors: **Friedrich Wolfsgruber**, Tacherting;  
**Hans W. Kasel**,  
Saarbrücken-Bischmisheim; **Manfred H. A. Odendahl**,  
Saarbrücken-Brebach; **Wolfram W. Mörsdorf**,  
Saarbrücken-Bischmisheim, all of Fed. Rep. of Germany

[73] Assignees: **SKW Trostberg Aktiengesellschaft**,  
Trostberg; **Halbergerhütte GmbH**,  
Saarbrücken, both of Fed. Rep. of Germany

[21] Appl. No.: **90,719**

[22] Filed: **Nov. 2, 1979**

[30] Foreign Application Priority Data

Nov. 3, 1978 [DE] Fed. Rep. of Germany ..... 2847787  
Oct. 9, 1979 [DE] Fed. Rep. of Germany ..... 2940946

[51] Int. Cl.<sup>3</sup> ..... C22C 33/08  
[52] U.S. Cl. ..... 75/130 R; 75/53;  
75/257

[58] Field of Search ..... 75/53, 130 R, 257

[56]

References Cited

U.S. PATENT DOCUMENTS

|           |         |                 |        |
|-----------|---------|-----------------|--------|
| 3,318,687 | 5/1967  | Bowden .....    | 75/53  |
| 3,649,248 | 3/1972  | Ishimitsu ..... | 75/257 |
| 3,669,618 | 6/1972  | Cappel .....    | 75/257 |
| 3,726,665 | 4/1973  | Minnick .....   | 75/257 |
| 3,771,999 | 11/1973 | Fedock .....    | 75/257 |
| 3,793,006 | 2/1974  | Kawawa .....    | 75/257 |
| 3,802,865 | 4/1974  | Ohkubo .....    | 75/53  |

Primary Examiner—P. D. Rosenberg

Attorney, Agent, or Firm—Sughrue, Rothwell, Mion, Zinn and Macpeak

[57]

ABSTRACT

A slow fade cast iron inoculant is made up of  
(a) a silicon-containing matrix of iron silicon alloys  
and having a crystal structure,  
(b) compounds, present in the matrix crystal structure,  
of high-melting point calcium aluminum silicates,  
generally in the form  $\text{CaO} \cdot \text{Al}_2\text{O}_3 \cdot 2\text{SiO}_2 + \text{Al}_2\text{O}_3 \cdot 2\text{SiO}_2$ , and  
(c) a dicalcium aluminum silicate material with up to  
20% by weight of silicon carbide and 10% by  
weight of calcium carbide.

The relation between the matrix and the high-melting point calcium aluminum silicates to the dicalcium silicate material is about 1 to 0.05–0.2. The amount of high-melting point calcium aluminum silicates in the matrix is 5 to 30% by weight and, more specially 8 to 15% by weight.

14 Claims, 12 Drawing Figures





**Fig. 2**

White-solidifying tendency in an induction furnace  
against time with and without addition of inoculant



4.  
High.

scatter of figures  
for supercooling



***Fig. 5***









**Fig. 10**

**Fig. 11**

***Fig. 12***

## SLOW FADE INOCCULANT AND A PROCESS FOR THE INOCCULATION OF MELTED CAST IRON

### BACKGROUND OF THE INVENTION

The present invention is with respect to an inoculant for processing cast iron and a process for use of the inoculant.

By definition the amount of carbon in cast iron is greater than 1.7%, small amounts of manganese, phosphorus, sulfur and silicon being present as well. When melted cast iron becomes solid, a part of the carbon is segregated out as graphite (in the case of gray cast iron) or as  $Fe_3C$  (cementite, in the case of white cast iron). The sort and amount of the impurities and other substances in the iron together with the selection of the rate of cooling, as dependent on the thickness of the casting on hand, have different effects on the solidification of the casting. Because white-solidified cast iron may not be readily machined because of its hardness and brittleness, white solidification is undesired for most uses and is stopped or limited by inoculation of the melted iron.

The inoculant which has been most widely and longest used is ferrosilicon with about 75% of silicon. Its effect is produced not only by the graphitizing caused by its silicon, but, to a great degree, certain controlled amounts of aluminum and calcium. The effect may be further increased by other materials such as barium, zirconium and strontium.

Other normally used inoculants are 30/60 calcium-silicon, mixed ferrosilicon and calciumsilicon and, furthermore, graphite.

It may be generally said that the inoculation of liquid metals is the placing of impurity nuclei in the melted material, which take the form of crystallization centers for the forming of graphite. In this respect, the inoculation effect is said to be caused only by solid crystallization nuclei. For this purpose substances with metallic, and furthermore substances with non-metallic properties, as for example oxides, sulfides, nitrides, borides and carbides may be used, while compounds which are broken down under the effect of heat, go into solution in the melted material or undergo reduction or decomposition may not be used as inoculants.

Generally speaking, there are two forms of inoculation: first-stage inoculation in the ladle as a single-stage process and first-stage inoculation in the ladle together with later, second-stage inoculation right before teeming or solidifying of the melt in the mold.

The overall amount of inoculant used is between about 0.1 and 0.8% by weight. With such amounts white-solidification of the cast iron may be stopped or limited to the desired degree, nucleation of the melt may be made better and graphite crystallization helped. However, such conditions are not without a parallel effect on the properties of the completed casting: With an increase in the amount of inoculant, undesired properties are produced, such as a decrease in hardness, an increase in blowholes, porosity, greater cracking, thicker flaking of graphite, amongst others.

### SHORT OVERVIEW OF THE PRESENT INVENTION

For this reason, attempts have been made at the development of nucleating melt inoculants keeping their effect for a longer time, that is to say low fade inoculants. For example the German Auslegeschrift specification No. 1,758,004 has a suggestion for a fine-grain,

synthetic silicon dioxide as such a melt inoculant or addition. However, judging from attempts at making use of this invention for normal works use, it does not seem that this inoculant has any low fade properties.

One purpose of the present invention is the development of a low fade inoculant, that is to say one which keeps its properties for a long time, for cast iron in a melting furnace or in an apparatus for keeping it hot. A further purpose of the present invention is that of decreasing greatly the amount of inoculant needed for the later inoculant addition itself.

The present invention is based on an inoculant for melted cast iron and, in the invention, this inoculant is characterised in that it is made up of

- 15 (a) a silicon-containing matrix of iron silicon alloys and having a crystal structure,
- (b) compounds, present in the matrix crystal structure, of high-melting point calcium aluminum silicates generally of the form  $CaO \cdot Al_2O_3 \cdot 2SiO_2 + 3Al_2O_3 \cdot 2SiO_2$ ,
- (c) a dicalcium aluminum silicate material with up to 20% by weight of silicon carbide and 10% by weight of calcium carbide.

in which respect the relation of the calcium-containing matrix with the high-melting point calcium aluminum silicates to the dicalcium silicate material is about 1 to 0.05-0.2 and the amount of high-melting point calcium aluminum silicates in the silicon-containing matrix is 5 to 30% by weight and more specially 8 to 15% by weight.

The amount of inoculant to melted cast iron may be 0.05 to 1% by weight or, more specially, 0.1 to 0.5% by weight.

The addition of the inoculant to the cast iron may take place in the melting apparatus, in and before the apparatus for keeping the cast iron hot or in the forehearth.

Furthermore the inoculant addition may be made to the burden or part of the burden before melting in an amount of 0.05 to 4% by weight.

In the case of producing cast iron with nodular or vermicular graphite by conditioning the melted iron with magnesium and/or rare earth metals, an addition is made, right before this conditioning, of a further amount of inoculant in an amount of 0.1 to 0.7% by weight and, more specially 0.2 to 0.4% by weight.

Surprisingly, the purpose of the invention is effected with an inoculant as noted or a process for inoculation as given.

It has been seen from tests that the inoculants of the present invention put an end to the shortcomings as noted of past inoculants and keep up the nucleating property of cast iron melt even at high temperatures (1150° C.), even if such temperatures are kept to for over 3 hours. For this reason, the different tendency of the melt to undergo white-solidification (on casting) in the furnace is decreased to a lower limiting value, at which it is kept unchangingly for more than 3 hours.

Generally, normal inoculation before teeming or on teeming may be limited to very small amounts of inoculant, which are at the same level for each tapping operation. The small amounts of inoculants of, for example 0.05 to 0.1% by weight, make it possible to get an unchanging end level of silicon in the melt, so that it is possible to keep to tighter tolerances in the different properties of the cast iron, which is then of an unchanging quality.

In a cast iron melting works using line frequency crucible furnaces, the tendency to white-solidification is measured on a sample and to get the best graphitizing effect, adjustment takes place by additions of inoculant. In the case of furnaces for some tonnes of metal, from which, on each tapping operation, only a little melt is run off, so that some hours may go by before all metal has been cleared from the furnace, there is, however, a smoothly increasing tendency to white-solidification. This may be overcome by increasing amounts of inoculant on tapping. The castings will then have different silicon levels, this having an effect on the behavior on teeming and furthermore the material properties of the castings will become less good for every increase in the amount of inoculant.

On the other hand, the low fade inoculant of the present invention makes it possible for the white-solidification tendency of the melt to be kept unchanging at a low level so that, on teeming, only further conditioning with small, unchanging amounts of inoculant are necessary. For this reason there are less changes in the solidification behavior of the cast iron and its quality from one tapping operation to the next one.

The inoculant of the present invention is made up of two substances with different effects. One of these substances is the iron silicon alloy, which, as is part of knowledge in the art, has the effect of producing the inoculated condition of the cast iron melt at once, and lastly, the low-fade inoculant itself, made up of high-melting point calcium aluminum silicates ( $\text{CaO} \cdot \text{Al}_2\text{O}_3 \cdot 2\text{SiO}_2 + \text{Al}_2\text{O}_3 \cdot 2\text{SiO}_2$ ), the dicalcium silicate material, silicon carbide and calcium carbide. These substances make it possible for the nucleation condition of the inoculated melt to be kept up for a long time. It has turned out to be useful if the dicalcium silicate material make up about 5 to 20% by weight of the iron silicate material and calcium aluminum silicate together. The level of the calcium aluminum silicate together. The level of the calcium aluminum silicate is to be between about 5 and 30% by weight of the iron silicon alloy. A specially good effect is produced if the percentage by weight is roughly 8 to 15.

For producing cast iron with nodular or vermicular graphite, nodulating materials such as magnesium and/or rare earth metals are used. The process of the present invention has turned out to be useful for producing such cast iron, in which respect, while it is true that the addition of magnesium or the like has the effect of increasing the tendency to white-solidification, the tendency is not as marked as is the case with melts not conditioned by using the present invention. It is only in this case, as part of a further development of the invention, that a further conditioning of the melt after being processed with magnesium or the like, has to take place using the inoculant of the present invention in amounts equal to 0.1 to 0.7% by weight and, more specially 0.2 to 0.4% by weight.

In this respect small amounts of inoculant of the present invention are enough. Further inoculation, after processing with magnesium or the like, with the inoculant of the present invention is, for this reason, a step usefully rounding off and completing the inoculation of the melt undertaken in the present invention in the first place.

It is not possible to say that this further inoculation is, in any way, like the addition of purely deoxidizing material (such as ferrosilicon), because the addition of the inoculant of the present invention is not only

sponsible for deoxidation, but furthermore is responsible for producing thermally stable nuclei in the melt, this making certain of a low fade rate after inoculation, that is to say the inoculation effect is kept up for a long time.

This further development of the process of the invention makes possible casting times of 20 minutes and longer, nodular graphite or vermicular graphite structure castings of an even, high quality being produced.

Inoculation into the mold or on teeming, only makes necessary very small amounts, the same in all cases, of inoculant which make certain of, generally speaking, unchanging physical properties of the castings because the behavior on solidification is the same in all cases.

With this further development of the process of the invention making use of smaller amounts of inoculant the number of solidification blowholes is decreased to the lowest possible level, that is to say the level possible in nodular graphite cast iron.

It is furthermore possible to see from the solidification behavior of such melts using the first and second differential coefficients of the cooling curve  $dT/dt$  and  $d^2T/dt^2$ , the relation between time and the heat of crystallization with respect to the nucleated condition, the supercooling temperature, the forming of graphite and blowholing, that such melts are markedly different to melts processed, for example, with 0.8% FeSi.

In the case of an unchanged chemical makeup, the higher the latent heat of formation  $L$  or the heat of crystallization  $Q$ , measured in J/g, the greater the amount of graphite which is segregated out between the solidus and liquidus temperature and has the effect of decreasing blowholes. The melts conditioned with this form of the process of the invention furthermore have the best possible feeding properties, a low tendency with respect to forming blowholes and the condition that the maximum of the second differential coefficient of the cooling curve against time is generally in line with the limiting value for vermicular graphite-forming.

Furthermore, with such conditioned melts, the curve of the relation between time and heat of crystallization is marked by a wide primary austenite range with the forming of a fine primary dendrite network with small graphite nodules and a generally flat curve path in the range of the eutectic heat of crystallization, so that the rest of the melt is kept in a liquid condition for a long time, teeming and feeding properties into the molds are made better and there is a high feeding efficiency.

#### LIST OF FIGURES

Some examples will now be given of the invention, which, however, are not to have the effect of limiting the invention in any way.

FIG. 1 is a graph of the white-solidifying tendency in an induction furnace against time in the case of the use of a normally used inoculant.

FIG. 2 is a graph of the white-solidifying tendency in an induction furnace against time, with and without the addition of the inoculant of the present invention.

FIG. 3 is a graph with respect to scatter of supercooling figures in the case of normally conditioned cast iron.

FIG. 4 is a graph with respect to case iron processed using the present invention.

FIG. 5 is a graph of the scatter in the figures for heat of crystallization of the melt in the ladle in the case of normally processed cast iron.

FIG. 6 is a graph on the same lines as figure with respect to teeming.

FIG. 7 is a graph of the scatter range of the heat of crystallization of the melt in the ladle in the case of cast iron conditioned with the present invention.

FIG. 8 is a graph on the same lines with respect to teeming.

FIG. 9 is a graph of the scatter range of the maximums of the second differential coefficient of the temperature/time curve in the ladle in the case of cast iron processed normally.

FIG. 10 is a graph on the same lines, but with respect to teeming.

FIG. 11 is a graph of the scatter range of the maximums of the second differential coefficient of the temperature/time curve in the ladle in the case of cast iron processed in the present invention, and

FIG. 12 is a graph on the same lines, but with respect to teeming.

#### EXAMPLES OF THE INVENTION

##### EXAMPLE 1 (comparison example, cast iron with flake graphite)

The reference makeup or analysis and temperature of melted cast iron underwent adjustment in a line frequency induction crucible furnace or apparatus for keeping the material hot, the apparatus having a buffer function. Even although there were no changes in the analysis and the temperature, the white-solidification tendency of the melt (measured in the form of white-solidification in a cast wedge) underwent changes.

Without being dependent on the tendency to white-solidification of the cast iron in the furnace at the start, this tendency became higher the longer the cast iron was kept in the apparatus for keeping it hot, this making necessary adjustment with ever increasing amounts of inoculant on teeming (for example up to 0.5%). The castings had:

- a great number of eutectic cells,
- coarse A-graphite,
- high tensile strength,
- many blowholes,
- a tendency to porosity,
- a low hardness,
- a high percentage of reaction products (slag).

The material properties of these castings are presented in table 1.

On keeping the metal in a melted condition for a longer time, making necessary greater additions of inoculant, these properties became worse.

##### EXAMPLE 2 (comparison example—cast iron with flake graphite)

Using normally marketed inoculants, an attempt was made at decreasing the tendency of cast iron to white-solidification, while the iron was still in an induction crucible furnace or apparatus for keeping it melted, to a lower limiting value and, in so doing, decreasing the amount of inoculant on teeming to 0.1% at the most, so that it would be possible to have a generally unchanging end-level of silicon and an unchanging quality of the cast iron.

As will be seen from FIG. 1, it was not possible for the inoculation effect to be stretched out to a time greater than 3 hours (as had been desired), and in fact the effect had faded away after 30 minutes at the most. The white-solidification tendency of the melt had to undergo adjustment by amounts of inoculant the same as in normal processing (table 2).

##### EXAMPLE 3 (flake graphite cast iron)

By the addition of the slow fade inoculant of the present invention in an induction crucible furnace or apparatus for keeping the metal in a melted condition, an unchanging level of white-solidification was kept up for 3 hours and longer (FIG. 2).

In this respect, for evening out the solidification behavior, small, unchanging amounts of inoculant of about 0.1% on tapping were enough. The casting produced had:

- a small number of eutectic cells,
- fine A-graphite structures
- a high enough strength,
- a low number of blowholes,
- a small amount of reaction products (table 3).

##### EXAMPLE 4 (comparison example—nodular graphite cast iron)

Although having the same analysis and temperature, charges of melted cast iron were produced in a low frequency crucible furnace at different levels of the tendency to white-solidification, this being measured in the form of supercooling or as the degree of white-solidification in cast wedges. The longer the time the material was kept melted, the greater the tendency to white-solidification (FIG. 3).

On keeping the metal for two hours in an induction furnace at 1550° C., there was an increase in white-solidification from 2.5 to 5 mm and in supercooling from 4 to 10.5° C. After conditioning with magnesium, the white-solidification tendency was 12 mm and supercooling 28° C. By an inoculation with 0.8% by weight of FeSi 75, the white-solidification tendency and supercooling went down to 3.5 mm and 6.5° C. in the ladle and went up till at the end of teeming after 20 minutes they had levels of 6 mm and 13° C. (table 4, FIG. 3).

The heat of crystallization was, at the start of teeming, 265 J/g and at the end of teeming 260 J/g, while the maxima of the second differential coefficient were 0.20 and, in the other case, 0.15° C./sec<sup>2</sup> (table 4; FIGS. 5, 6, 9 and 10).

In order to make possible teeming of cementite-free castings at the end of the teeming operation with a degree of supercooling of 13° C. and a white-solidification tendency of 6 mm, inoculation on teeming with 0.1% by weight of inoculant was necessary. Although, in this case, the white-solidification tendency of the melt went down to 2.5 mm at the start and 3.0 mm at the end and supercooling went down to 1.5° C. and 2.5° C., the heat of crystallization going up by 5 J/g to only 268 J/g at the start and 265 J/g at the end of the teeming time, the maxima of the second differential coefficient kept the same at 0.19° C./sec<sup>2</sup> (table 4).

Such melted cast iron has:

- a high value for the supercooling temperatures and a high white solidification tendency at the end of teeming before teeming inoculation
- lower heats of crystallization undergoing greater changes and a low self-feeding property (FIGS. 5 and 6)
- lower maxima of the second differential coefficient  $d^2T/dt^2$  of the cooling curve against time and a worse feeding property (FIGS. 9 and 10).

## EXAMPLE 5 (nodular graphite cast iron)

Melted cast iron, conditioned as in example 3, had, even after being kept for 2 hours and longer in a melted condition in an induction furnace, a white-solidification tendency of under 3 mm and supercooling values of under 5° C. (see FIG. 4 and table 5). White-solidification tendency and supercooling went up after magnesium conditioning have as well (9 mm, 21.5° C.). The melt was inoculated right after magnesium processing with 0.3% by weight of the inoculant given in example 3. Over the full time of 20 minutes, the values for the white-solidification tendency and supercooling kept generally unchanged at 4 mm and 8.0° C. In this respect the amounts of inoculant for teeming and in-mold inoculation were 0.03% by weight (for example in the form of FeSi) for stopping the coming into existence of primary cementite.

The conditioning of the melt, of which an account has been given, will make it clear that for the whole teeming time of the charge, the heats of crystallization were 10 J/g higher than in the comparison example 1; the maxima of the second differential coefficient kept unchanged at about 0.4° C./sec<sup>2</sup> and, for this reason, were twice as high as in the comparison example 1, that is to say near the transition to vermicular graphite (table 5, FIGS. 7, 8, 11 and 12).

The further teeming inoculation with 0.03% by weight of FeSi 75 put up the heats of crystallization once again by 5 J/g, while the maxima of the second differential coefficient were still 0.4° C./sec<sup>2</sup> (table 5, FIGS. 7, 8, 11, 12).

So the effects produced are:

a low and unchanging level of supercooling and the tendency to white solidification of the melt for the teeming time before teeming inoculation

high heats of crystallization with a low scatter even before teeming inoculation, that is to say good self-feeding conditions (FIGS. 7 and 8)

high, unchanging values for the maximum of the second differential coefficient of the cooling curve against time and better feeding properties (FIGS. 11 and 12).

The same effects may be produced on using the process of the invention for vermicular graphite cast iron.

We claim:

1. An inoculant for melted cast iron comprising:
  - (a) a silicon-containing matrix of iron-silicon alloys and having a crystal structure,
  - (b) a high-melting point calcium aluminum silicate compound, present in the matrix crystal structure, and

(c) a dicalcium aluminum silicate material with up to 20% by weight of silicon carbide and up to 10% by weight of calcium carbide,

the weight ratio of the calcium-containing matrix with the high-melting point calcium aluminum silicate to the dicalcium silicate material being about 1:0.05 to about 1:0.2 and the amount of high-melting point calcium aluminum silicate in the silicon-containing matrix being 5 to 30% by weight.

2. The inoculant of claim 1, wherein said high-melting point calcium aluminum silicate is  $\text{CaO} \cdot \text{Al}_2\text{O}_3 \cdot 2\text{SiO}_2 + 3\text{Al}_2\text{O}_3 \cdot 2\text{SiO}_2$ .

3. The inoccculant of claim 1, wherein the amount of high-melting point calcium aluminum silicate in the silicon-containing matrix is 8 to 15% by weight.

4. A process for the inoculation of melted cast iron, comprising adding an inoculant as claimed in claim 1 in an amount of 0.05 to 1% by weight to the melted cast iron.

20 5. A process as claimed in claim 4, comprising adding said inoculant in an amount of 0.1 to 0.5% by weight.

6. A process as claimed in claim 4 or claim 5, comprising adding said inoculant to the cast iron in an apparatus for keeping it in a melted condition, in and before 25 the apparatus or to the melted cast iron in the forehearth.

7. A process as claimed in claim 4 or claim 5, comprising adding said inoculant to the burden or a material of the burden before melting, in an amount of 0.05 to 4% by weight.

30 8. A process as claimed in claim 4 or claim 5, said process producing nodular or vermicular graphite cast iron by conditioning melted cast iron with magnesium and/or rare earth elements and said process comprising, right after this conditioning step, further adding said inoculant in amount of 0.1 and 0.7% by weight.

9. A process as claimed in claim 6, said process producing nodular or vermicular graphite cast iron by conditioning melted cast iron with magnesium and/or 40 rare earth elements and said process comprising, right after this conditioning step, further adding said inoculant in amount of 0.1 and 0.7% by weight.

10. A process as claimed in claim 7, said process producing nodular or vermicular graphite cast iron by 45 conditioning melted cast iron with magnesium and/or rare earth elements and said process comprising, right after this conditioning step, further adding said inoculant in amount of 0.1 and 0.7% by weight.

11. A process as claimed in claim 8, wherein the 50 amount of the inoculant is 0.2 to 0.4% by weight.

12. A process as claimed in claim 9, wherein the amount of the inoculant is 0.2 to 0.4% by weight.

13. A process as claimed in claim 10, wherein the amount of the inoculant is 0.2 to 0.4% by weight.

55 14. A process as claimed in claim 11, wherein the amount of the inoculant is 0.2 to 0.4% by weight.

\* \* \* \* \*

UNITED STATES PATENT AND TRADEMARK OFFICE  
CERTIFICATE OF CORRECTION

PATENT NO. : 4,292,075  
DATED : September 29, 1981

Page 1 of 6

INVENTOR(S) : Friedrich Wolfsgruber et al

It is certified that error appears in the above-identified patent and that said Letters Patent is hereby corrected as shown below:

Column 1, line 13, delete the first occurrence of "cast" and substitute therefor --case--.

Column 3, lines 37-38, delete the sentence fragment "The level of the calcium aluminum silicate together.".

Column 5, between lines 46 and 47, insert the following:

TABLE 1: normal processing

| Tendency<br>to white-<br>solidifi-<br>cation in<br>the induc-<br>tion fur-<br>nace | Addition<br>of inocu-<br>lant in<br>induction<br>furnace | Tendency<br>to white-<br>solidifi-<br>cation in<br>the induc-<br>tion fur-<br>nace | Addition<br>of inocu-<br>lant out-<br>side<br>furnace | white-<br>solidifi-<br>cation<br>tendency<br>on tap-<br>ping | material properties |                  |               |   |   |                       |                         | analysis                                |      |                    |               |      |      |     |
|------------------------------------------------------------------------------------|----------------------------------------------------------|------------------------------------------------------------------------------------|-------------------------------------------------------|--------------------------------------------------------------|---------------------|------------------|---------------|---|---|-----------------------|-------------------------|-----------------------------------------|------|--------------------|---------------|------|------|-----|
|                                                                                    |                                                          |                                                                                    |                                                       |                                                              | HB                  | G <sub>B</sub>   | graphi-<br>te |   |   | gra-<br>phite<br>size | base-<br>struc-<br>ture | aut.<br>cells<br>per<br>cm <sup>3</sup> | C    | Si<br>furna-<br>ce | Si<br>chunk   | Mn   | S    | Cr  |
| mm                                                                                 | %                                                        | mm                                                                                 | %                                                     | mm                                                           | $\frac{N}{mm^2}$    | $\frac{N}{mm^2}$ | %             | % | % | %                     | %                       | %                                       | %    | %                  | %             | %    | %    | %   |
| 5,0                                                                                |                                                          | 5,0                                                                                | 0,5                                                   | 2,0                                                          | 207                 | 297              | 100           | - | - | 4-6                   | 100%<br>Perlit          | 700                                     | 3,35 | 1,60               | 1,90-<br>2,20 | 0,80 | 0,08 | 0,2 |

UNITED STATES PATENT AND TRADEMARK OFFICE  
CERTIFICATE OF CORRECTION

PATENT NO. : 4,292,075

Page 2 of 6

DATED : September 29, 1981

INVENTOR(S) : Friedrich Wolfsgruber et al

It is certified that error appears in the above-identified patent and that said Letters Patent is hereby corrected as shown below:

Column 5, after line 68, insert the following:

TABLE 2: Use of normal inoculants in induction furnace

| Tendency<br>to white-<br>solidifi-<br>cation in<br>the induc-<br>tion<br>furnace | Addition<br>of inocu-<br>lant in<br>induction<br>furnace | Tendency<br>to white-<br>solidifi-<br>cation in<br>the induc-<br>tion<br>furnace | Addition<br>of inocu-<br>lant out-<br>side<br>furnace | white<br>solidifi-<br>cation<br>tendency<br>on<br>tapping | material properties |                  |               |    |    |                         | analysis                                |     |                    |             |               |      |      |     |
|----------------------------------------------------------------------------------|----------------------------------------------------------|----------------------------------------------------------------------------------|-------------------------------------------------------|-----------------------------------------------------------|---------------------|------------------|---------------|----|----|-------------------------|-----------------------------------------|-----|--------------------|-------------|---------------|------|------|-----|
|                                                                                  |                                                          |                                                                                  |                                                       |                                                           | NB                  | G <sub>B</sub>   | gra-<br>phite |    |    | base-<br>struc-<br>ture | eut.<br>cells<br>per<br>cm <sup>3</sup> | t   | Si<br>fur-<br>nace | Si<br>chunk | Mn            | S    | Cr   |     |
|                                                                                  |                                                          |                                                                                  |                                                       |                                                           |                     |                  | A             | B  | D  |                         |                                         |     |                    |             |               |      |      |     |
| mm                                                                               | %                                                        | mm                                                                               | %                                                     | mm                                                        | $\frac{N}{mm^2}$    | $\frac{N}{mm^2}$ | /%            | /% | /% |                         | /%                                      |     | /%                 | /%          | /%            | /%   | /%   |     |
| 6,0                                                                              | 0,3                                                      | 5,5                                                                              | 0,5                                                   | 3,0                                                       | 191                 | 279              | 100           | -  | -  | 4-5                     | 100%<br>Perlit                          | 600 | 3,35               | 1,40        | 1,00-<br>2,20 | 0,80 | 0,08 | 0,2 |

Column 6, between lines 19 and 20, insert the following:

UNITED STATES PATENT AND TRADEMARK OFFICE  
CERTIFICATE OF CORRECTION

PATENT NO. : 4,292,075

Page 3 of 6

DATED : September 29, 1981

INVENTOR(S) : Friedrich Wolfsgruber et al

It is certified that error appears in the above-identified patent and that said Letters Patent is hereby corrected as shown below:

TABLE 3: Use of inoculant of the present invention in induction furnace

| Tendency<br>to white-<br>solidifi-<br>cation in<br>the induc-<br>tion fur-<br>nace | Addition<br>of inocu-<br>lant in<br>induction<br>furnace | Tendency<br>to white-<br>solidifi-<br>cation in<br>the induc-<br>tion fur-<br>nace | Addition<br>of inocu-<br>lant out-<br>side<br>furnace | white<br>solidifi-<br>cation<br>tendency<br>on<br>tapping | material properties |                    |               |    |    |                         | analysis |                 |                                      |      |      |      |      |      |
|------------------------------------------------------------------------------------|----------------------------------------------------------|------------------------------------------------------------------------------------|-------------------------------------------------------|-----------------------------------------------------------|---------------------|--------------------|---------------|----|----|-------------------------|----------|-----------------|--------------------------------------|------|------|------|------|------|
|                                                                                    |                                                          |                                                                                    |                                                       |                                                           | HB                  | G <sub>B</sub>     | gra-<br>phite |    |    | base-<br>struc-<br>ture |          |                 | eut.<br>cells<br>per cm <sup>3</sup> | %    | %    | %    |      |      |
|                                                                                    |                                                          |                                                                                    |                                                       |                                                           |                     |                    | A             | B  | O  | VZ                      | 4-6      | 100 %<br>PERLIT |                                      |      |      |      |      |      |
| mm                                                                                 | mm                                                       | mm                                                                                 | mm                                                    | mm                                                        | kg/mm <sup>2</sup>  | kg/mm <sup>2</sup> | /%            | /% | /% | —                       | —        | —               | 450                                  | 3,35 | 1,70 | 1,90 | 0,80 | 0,08 |
| 5,5                                                                                | 0,3<br>LZI                                               | 3,5                                                                                | 0,1                                                   | 2,5                                                       | 201                 | 262                | 100           | —  | —  | VZ                      | 4-6      | 100 %<br>PERLIT |                                      |      |      |      |      | 0,2  |

Column 6, line 24, delete "cricible" and insert

therefor --crucible--.

Column 6, between lines 45 and 46, insert the  
following:

UNITED STATES PATENT AND TRADEMARK OFFICE  
CERTIFICATE OF CORRECTION

PATENT NO. : 4,292,075  
DATED : September 29, 1981

Page 4 of 6

INVENTOR(S) : Friedrich Wolfsgruber et al

It is certified that error appears in the above-identified patent and that said Letters Patent is hereby corrected as shown below:

Table 4

| Last charge of a furnace                                                          | Induction furnace | after magnesium processing | start of charge | ladle | end of charge | start of teeming charge | end of teeming charge |
|-----------------------------------------------------------------------------------|-------------------|----------------------------|-----------------|-------|---------------|-------------------------|-----------------------|
| White solidification (mm)                                                         | 5,0               | 12,0                       | 3,5             | 6,0   |               | 2,5                     | 3,0                   |
| Supercooling (°C)                                                                 | 10,5              | 28,0                       | 6,5             | 13,0  |               | 1,5                     | 2,5                   |
| heat of crystallisation (J/g) (1250°C)                                            | -                 | -                          | 265             | 260   |               | 268                     | 265                   |
| Maximum of second differential coefficient (°C/sec²) ( $\frac{dT}{dt}$ ) (1250°C) | -                 | -                          | 0,20            | 0,15  |               | 0,19                    | 0,19                  |
| Temperature (°C)                                                                  | 1550              | 1450                       | 1410            | 1360  |               | -                       | -                     |
| Carbon (%)                                                                        | 3,78              | 3,78                       | 3,78            | 3,78  |               | 3,78                    | 3,78                  |
| Magnesium (%)                                                                     | -                 | 0,045                      | 0,042           | 0,040 |               | 0,040                   | 0,039                 |
| Silicon (%)                                                                       | 1,90              | 1,90                       | 2,45            | 2,45  |               | 2,45                    | 2,45                  |
| Phosphorus (%)                                                                    | 0,056             | 0,055                      | 0,056           | 0,056 |               | 0,056                   | 0,055                 |
| Sulfur (%)                                                                        | 0,010             | 0,009                      | 0,009           | 0,009 |               | 0,009                   | 0,009                 |
| Manganese (%)                                                                     | 0,30              | 0,30                       | 0,30            | 0,30  |               | 0,30                    | 0,30                  |
| Chromium (%)                                                                      | 0,02              | 0,02                       | 0,02            | 0,02  |               | 0,02                    | 0,02                  |

UNITED STATES PATENT AND TRADEMARK OFFICE  
CERTIFICATE OF CORRECTION

PATENT NO. : 4,292,075  
DATED : September 29, 1981

Page 5 of 6

INVENTOR(S) : Friedrich Wolfsgruber et al

It is certified that error appears in the above-identified patent and that said Letters Patent is hereby corrected as shown below:

Column 7, line 7, after the period and before

"White-solidifica-", insert the following:

Table 5

| Last charge of a furnace                                              | Induction furnace | after magnesium processing | ladle           |               | teeming         |               |
|-----------------------------------------------------------------------|-------------------|----------------------------|-----------------|---------------|-----------------|---------------|
|                                                                       |                   |                            | start of charge | end of charge | start of charge | end of charge |
| White solidification (mm)                                             | 3,0               | 9,0                        | 3,5             | 4,0           | 2,0             | 2,5           |
| Supercooling (°C)                                                     | 4,5               | 21,5                       | 5,7             | 8,0           | 0,7             | 1,3           |
| heat of crystallization (J/g (1250°C))                                | -                 | -                          | 275             | 270           | 280             | 274           |
| maximum of second differential coefficient (°C/sec²) (dT/dt) (1250°C) | -                 | -                          | 0,42            | 0,38          | 0,43            | 0,40          |
| Temperature (°C)                                                      | 1550              | 1440                       | 1405            | 1350          | -               | -             |
| Carbon (%)                                                            | 3,78              | 3,78                       | 3,78            | 3,78          | 3,78            | 3,78          |
| Magnesium (%)                                                         | -                 | 0,042                      | 0,040           | 0,038         | 0,038           | 0,037         |
| Silicon (%)                                                           | 2,05              | 2,05                       | 2,21            | 2,21          | 2,23            | 2,23          |
| Phosphorus (%)                                                        | 0,055             | 0,055                      | 0,056           | 0,055         | 0,056           | 0,056         |
| Sulfur (%)                                                            | 0,008             | 0,008                      | 0,007           | 0,008         | 0,007           | 0,007         |
| Manganese (%)                                                         | 0,30              | 0,30                       | 0,30            | 0,30          | 0,30            | 0,30          |
| Chromium (%)                                                          | 0,03              | 0,03                       | 0,03            | 0,03          | 0,03            | 0,03          |

UNITED STATES PATENT AND TRADEMARK OFFICE  
CERTIFICATE OF CORRECTION

PATENT NO. : 4,292,075

Page 6 of 6

DATED : September 29, 1981

INVENTOR(S) : Friedrich Wolfsgruber et al

It is certified that error appears in the above-identified patent and that said Letters Patent is hereby corrected as shown below:

Column 7, line 51 (line 1 of Claim 1), delete  
"inocullant" and substitute therefor --inocculant--.

Signed and Sealed this

Fifth Day of April 1983

[SEAL]

Attest:

GERALD J. MOSSINGHOFF

Attesting Officer

Commissioner of Patents and Trademarks